

Aug. 20, 1963

C. SHEER ET AL

3,101,308

PROCESS FOR REDUCTION OF ORES TO METALS, ALLOYS, INTERSTITIAL  
AND INTERMETALLIC COMPOUNDS

Filed Oct. 11, 1960

REDUCTION FROM METAL OXIDE ONLY



INVENTORS  
CHARLES SHEER  
SAMUEL KORMAN  
BY JAMES O. GIBSON

*Willis B. Rice*  
ATTORNEY

## 1

3,101,308

**PROCESS FOR REDUCTION OF ORES TO METALS, ALLOYS, INTERSTITIAL AND INTERMETALLIC COMPOUNDS**

Charles Sheer, Teaneck, N.J., Samuel Korman, Hewlett, N.Y., and James O. Gibson, New Providence, N.J., assignors to Sheer-Korman Associates, Inc., New York, N.Y., a corporation of Delaware

Filed Oct. 11, 1960, Ser. No. 61,870

7 Claims. (Cl. 204—164)

This invention relates to a process for the carbothermic reduction of ores concentration of metal compounds particularly oxide compounds for the production of metal carbides, by the application of a hierarc in a new and unique manner. In this application the term "hierarc" is used to define a particular form of arc discharge whose gas discharge mechanism and basic properties are distinct from the conventional form of arc discharge commonly used today in electrochemistry.

The hierarc is established whenever a gas or vapor is caused to flow in appreciable amounts into the conduction zone of the arc from that portion of the surface of the anode which is enged in receiving current from the arc, i.e. which is serving as the positive electrode terminus of the discharge. Thus, in the vicinity of the electrode boundary, the gas or vapor flows against or in opposition to the flow of current, thereby exerting some form of aerodynamic influence on the stream of electrons and ions comprising the arc current.

The exact nature of this fluid mechanical gas-stream interaction with the arc current stream is as yet unknown. However, its effect on the characteristics of the arc discharge are quite profound. In particular it causes a radical shift in the manner in which the energy of the arc is concentrated.

For example, in the conventional arc discharge, the major portion (80—90%) of the energy input is dissipated uniformly within the conduction column between the anode and cathode, and escapes out the cylindrical sides of the column into the surrounding atmosphere by radiation, thermal conduction, and diffusion. The remainder of the input energy (10—20%) is transferred to the two electrodes at the current boundaries.

In the hierarc, however, the bulk of the energy dissipation (60—75%) is shifted to a very small region adjacent to the electrode boundary from which the gas is flowing. This energy focusing property results in the establishment of a much more highly concentrated energy zone within the discharge itself than can occur in any other known form of arc discharge. This in turn provides the basis for the achievement of either much higher temperatures or more rapid and efficient transfer of energy to the gas stream flowing through the zone and to the subjacent electrode boundary, or both, depending on easily controllable operating parameters. In such a situation only a minor fraction of the total energy dissipated now escapes the discharge site without first having been transferred to said gas stream and electrode.

The inventors have discovered that the energy focusing property is directly related to the passage of gas into the arc from the current-receiving electrode boundaries. The effect becomes very pronounced when the gas flow occurs in amounts sufficient to affect the electrical charge distribution in the conduction column. Under these conditions it is believed that the flow of gas particles is comparable in amount to the opposite flow of electrons which constitutes the arc current. Moreover, the change in arc characteristics, when the mode of operation changes from the conventional arc to that of the hierarc, occurs quite suddenly as the flow rate of gas from the electrode boundary approaches this value.

## 2

Since the effect is more easily established at the anode than at the cathode, the inventors have preferred to work with gas flow from the positive terminus of the discharge. The description of practical results below will therefore mention only the anode in connection with this phenomenon. It is to be understood, however, that either electrode may be used, or both, and that the arc may be operated either on D.C. or on single or polyphase A.C., during the conduct of this process. In summary, the hierarc is an arc discharge in which the bulk of the energy is concentrated in a very small zone adjacent to the electrode boundary of the discharge by reason of the flow of gas or vapor from said boundary when the rate of flow has been properly adjusted to the arc current.

In our first application of the hierarc to metallurgy we fabricated a carbon electrode containing the ore to be reduced, and we operated it as an anode in an electric arc. At a certain value of current density it was found that the surface of the anode reached a point where there was projected into the arc from the anode surface a copious stream of vapor. The latter consisted of vaporized anode material which issued from the arc at very high temperature and in highly ionized form. This stream we have called the tail flame. This material formed a high speed jet in which the constituents of the anode were present in elemental form. The process was operated in an atmosphere of chlorine to prevent the metals from reoxidizing as they cool.

This effect is very pronounced when the gas flow is in substantial amounts and it appears to reach its maximum when the flow of gas particles from the anode is comparable to the flow of electrons which constitute the arc current. Moreover this transition from the common arc to the hierarc is quite sudden.

Upon first striking the arc, the passage of the current to the electrodes must first heat up the electrode surfaces at the contact interface. But then suddenly, when the anode face reaches the boiling point of the anode material, the copious vapor stream bursts out, and the high concentration of energy transfer to the anode face characteristic of the hierarc is established.

There is moreover a marked maximum of reaction rate at the point where the number of particles of the anode material moving in the flame is commensurate with the opposing flux of electrical particles comprising the discharge current. That is the number of molecules per second leaving the anode per square centimeter of active anode crater should be of the same order of magnitude as the number of current-carrying electrons per second entering the same area.

In this first embodiment therefore the jet of material projected into the arc was obtained by utilizing the energy focusing property of the hierarc to vaporize the material of the anode itself. The anode face therefore was brought to the temperature of vaporization of the ore and carbon in the anode.

We also devised a different form in which the vapor necessary to establish the hierarc effect could be introduced into the anode sheath of the arc by using a porous or finely perforated anode and injecting the vapor through the pores of the anode. In this way the material to be reacted upon could be introduced into the arc as a gas and subjected to the intense energy concentration near the anode characteristic of the hierarc. At the same time the passage of the gas through the pores of the anode serves to keep the porous anode relatively cool, thus preventing the consumption of the porous anode structure itself. In this modification the external gas, rather than the vapor of the anode, provides the fluid mechanical interaction with the arc discharge which causes the arc operation to shift to the hierarc mode. The porous anode,

which is not consumed during operation, serves merely as a current collector.

Now the inventors have discovered still a third method of establishing a hierarc. This consists of promoting a chemical reaction at the surface of the anode such that at least one of the products is in the gaseous phase and issues from the active surface at a rate relative to the arc current sufficient to initiate the hierarc.

One of the distinctive features of this modification is that it no longer involves the requirement that the material of the anode at the face of the crater be raised to the vaporization point. This results from the fact that there are a large number of chemical reactions in which refractory products are formed which can occur between materials of the anode in the solid or liquid state, and which produce one or more products in the gaseous state. Further these reactions may be caused to proceed at practical rates even though the reacting partners are heated to temperatures considerably below the boiling points of the refractory products.

Finally, the experiments of the inventors have demonstrated that the rate at which the product gas can be evolved at such lower temperatures is sufficient to initiate and sustain the hierarc mode of operation, even when the arc current is too low to cause any appreciable vaporization of the anode constituents.

The accompanying diagram illustrates how the process has been carried out in practice.

In the drawings the refractory metal to be recovered is produced in liquid form, and as here shown, the energizing gas is CO. This is produced by the reaction between the ore, particularly the oxide ore, and carbon at the anode crater.

In this invention the energy applied to the anode is controlled or limited in such a manner that the vaporization point of at least one of the reaction products is not reached. This control can be attained by varying the rate of feed of current to the arc, or by varying the rate of rotation of the electrodes.

Referring now to the figure, the numeral 10 represents an electrode fabricated, for example, of columbium oxide with a stoichiometric quantity of carbon such as to reduce the metal to metallic form or to a carbide, and discharge the oxygen as CO gas. The numeral 11 is a brush or slideable contactor of some suitable kind, to connect the positive side 12 of a source of power with the electrode 10. The numeral 13 is a cathode, connected by a brush 14 with the negative side 15 of the source of power. The anode face 16 is of a larger area than the crater of the arc which is to be struck upon it, and as here shown the cathode is mounted to contact the anode face off center, preferably at a downwardly inclined angle above the center.

When the cathode first contacts the anode face the current flowing through the resistance of the contact raises the temperature of the local area of the anode face up to the point of thermal reduction of the metal oxide of the ore with the carbon present. This reaction produces carbon monoxide gas, which flows into the arc conduction column and interacts with the current, thus establishing the hierarc as soon as the contacts are separated. Thereafter, the hierarc effect may be maintained by the product carbon monoxide gas liberated continuously by the reduction reaction occurring at the anode surface, while the molten metal product drips off the anode as shown. It may be recovered as beads or "round shot," or it can be caused to fall into a molten bath.

The anode may be rotated about its axis, during the operation, in order to help control the temperature of the reaction zone upon the anode face, and to thus control the rate of reduction.

The process may be conducted in an atmosphere of argon or helium or in some cases where no interaction will occur, in an atmosphere of hydrogen or hydrocarbon.

The present invention is based on the use of the hierarc

principle to transfer energy to a reacting mixture such as, for example an oxide ore and carbon in order to produce either the metal or a metal carbide. Which of these two products is produced can easily be determined by adjustment of the carbon stoichiometry. This is illustrated in the following equations:



10 (where Me=any metal, assumed in this example to be divalent).

In Example 1 the product will be a metal and carbon monoxide, while in Example 2 the product is the metal carbide plus carbon monoxide. In both cases the reaction produces a product which is a gas, even at room temperatures; namely, carbon monoxide.

In carrying out this reaction, as in our earlier application, a consumable electrode is made containing the metal oxide and carbon in the required proportions, as indicated by Examples 1 and 2, and the arc is struck in a neutral or otherwise compatible atmosphere to avoid re-oxidation or contamination of the product. The ambient pressure during operation was found to be relatively non-critical as regards promoting the reduction. However, it was found that better control of the reaction and a purer product could be obtained by reduced pressure. For this reason the inventors prefer to operate at pressures in the range from 0.01 to 10 mm. of mercury although useful results may be achieved outside this range of pressures.

30 One of the important requirements for this process is that the reaction rate be sufficiently rapid so that (a) enough CO gas is generated to maintain the hierarc energy distribution and (b) the reaction is essentially complete before any of the constituent materials leave the anode and enter the arc. The reason for the first of these requirements is obvious in view of the previous discussion. The second requirement stems from the fact that if the reaction is incomplete before the reacting

40 components reach the arc crater the end product will be contaminated with unreacted starting materials.

In order to achieve the desired condition it is essential that the anode surface at the electrode-arc boundary be maintained at an appropriate temperature within a well defined range.

45 The lower limit of this range is prescribed by the requirements (a) and (b) above.

The existence of an upper limit was discovered during the experimental investigations of the inventors and arose for the following reason: When the surface temperature at the anode crater is raised beyond a certain point (which point may still be well below the vaporization temperature of the constituents) the thickness of the section of the electrode behind the anode crater which is hot enough to promote the carbothermic reduction increases. Consequently CO gas is generated at some depth within the body of the electrode. At sufficiently high temperatures the gas may be generated at a point too far from the crater surface to allow it to escape by diffusion at the rate at which it is generated.

60 When this occurs, the pressure of said product gas within the electrode begins to build up until it either shatters the electrode or splatters the molten film off the anode before the reaction is complete at that point, thus interrupting the process. The upper limit of surface temperatures during operation therefore is dictated by the particular characteristics of the ore being used and the product being produced. This obviously follows from the fact that the reaction rate for carbothermic reduction is a function of the temperature as well as the reaction rate constant for the particular materials involved. This constant is different for each ore, and for the same ore, is different for production of the metal than for the production of its carbide.

70 However, once the starting materials and products

are specified it is fairly simple to determine the practical limits of operation as regards surface temperature. All that is required is first to adjust the conditions of operation so that the surface temperature is high enough to produce the plasma tail flame of CO gas, which is easily visible and which is a sign that hierarc operation has been achieved, and secondly to increase the temperature beyond this point to the degree necessary to prevent unreacted ore from appearing in the product. This establishes the lower limit of surface temperature during operation.

The upper limit of the practical operating range is then determined by increasing the surface temperature until spalling of the electrode or splattering of the molten film occurs. The practical working range lies between these two limits.

It should be emphasized that, in contrast to our previous application, the reaction zone does not occur anywhere in the arc itself, but rather in a thin film of material across the tip of the electrode subjacent to the arc crater. Despite this fact, operation of the arc in the hierarc mode is essential to achieve the practical results the inventors have observed. They have noticed invariably that when the prevailing mode of operation is that of the conventional arc, i.e. when the rate of CO evolution from the surface is too low to cause the hierarc focusing effect, the rate of production becomes very small relative to the power expended, and the process becomes highly inefficient. Thus, when the latter condition obtains, the bulk of energy is not transferred to the reacting materials and is therefore not used in promoting the reaction. Instead it is wastefully dissipated.

Concurrently the inventors have found that the degree of contamination of the product, when the conventional type of arc operation is used, is far greater than when the hierarc is established.

A second important feature of this new technique is the discovery of the inventors that the optimum range of temperature for promoting the reaction in the manner described is generally such that one or more of the product materials involved is in the molten state. For example, referring to Examples 1 and 2 above, it is found that the metal or metal carbide exists in the molten state when the process is conducted within the optimum range of surface temperatures. Moreover, this range of temperatures is sufficiently wide so that an operating temperature may be selected at which the molten film at the anode face exerts negligible vapor pressure. At this temperature therefore the tip of the electrode is always covered with a thin film of molten metal or metal carbide through which the CO gas can easily diffuse without significant losses of the desired product.

As the reaction proceeds the thickness of the molten film, which adheres to the anode face initially by surface tension, becomes thick enough so that it agglomerates in the form of a droplet which detaches itself from the anode surface and falls under the action of gravity. In this manner the product automatically and continuously leaves the reaction zone so that the thickness of the molten film remains essentially constant while the reaction proceeds indefinitely. Moreover, if the length of fall provided for in the reaction chamber is sufficient, the droplet of metal or metal carbide will freeze before it strikes the bottom of the reaction chamber. Once frozen to the solid state the metallic bead is relatively inert and does not become contaminated by contact with the chamber wall.

This manner of operation has several extremely valuable properties; first, it permits the reduction reaction to be carried on continuously; secondly it provides for the removal of the product from the reaction zone in such a way as to avoid completely the possibility of any back reaction, so that quantitative yields can be obtained; and thirdly, by maintaining the proper surface temperature, the reduction reaction can be made to go to completion

before the droplet agglomerates and falls off the surface. Furthermore, if the droplet is allowed to freeze before striking the bottom, the product may be withdrawn from the chamber without ever having come in contact with the walls of a containing vessel while in the reactive molten state. This feature completely avoids one of the more baffling and difficult practical problems encountered in the field of metallurgy. This problem relates to the problem of the crucible required to contain the materials which is now universally used in competitive conventional techniques. In such processes vessel walls are invariably attacked by many molten metals or carbides especially for such elements as columbium, titanium, uranium, etc. When these materials come in contact with the container walls in the molten state, the melt attacks the crucible walls until the crucible is destroyed, and at the same time the product becomes contaminated with container material.

In the present process this problem is completely eliminated and the product is produced in the form of round shot of especially high purity.

A further advantage which may be noted at this point is that when the process is conducted at low ambient pressures, volatile impurities are expelled from the molten film while the material resides on the tip of the electrode. Thus, some of the purifying action characteristic of vacuum melting is secured by this technique simultaneously with the reduction process and without extra cost.

For example, in the production of columbium the following purification took place:

|                |           | P.p.m. |
|----------------|-----------|--------|
| In ore:        | Zirconium | 1000   |
|                | Si        | 1000   |
| 35 In product: | Zirconium | 200    |
|                | Si        | 100    |

It has also been found possible to regulate the size of the spheres of metal or metal carbide produced in this process by a slight variation in the conditions of operation. This is done by varying the operating surface temperature within the operating range described above.

At the lower limit of this range the liquid product accumulates in the form of relatively large droplets since the pressure of CO gas is produced sufficiently low so that it does not disturb the dripping process. As the surface temperature is raised slightly the pressure of CO gas within the molten film increases, and we have found that this has a tendency to cause the molten droplets to detach from the surface with smaller sizes.

At the upper extreme of the operating range, before the onset of excessive splatter or spalling within the electrode, the particles have been observed to blow off in the form of very small droplets in the fashion of a liquid atomizer. Thus, using a  $\frac{3}{4}$ " diameter anode it has been found possible to vary at will the size of the spheres produced from  $\frac{5}{16}$ " diameter down to as low as -325 mesh.

In the practical application of this process the inventors have varied two parameters in order to facilitate the achievement of the optimum temperature at the anode surface. One of these is the total arc current for a given electrode diameter, and the second is motion of the anode crater on the anode surface. Since in this modification of the process it is no longer necessary to cover the entire tip of the electrode, the arc current can be reduced until the arc terminus is considerably less than the diameter of the tip.

The inventors have found that if the electrode is rotated at the proper speed so that the arc terminus sweeps out the total electrode surface area, the entire electrode may be consumed while at the same time the average surface temperature obtaining over the surface may easily be adjusted over a wide range.

Typical examples of this process which have been worked out in the laboratory for each type of product are the following:

(A) *Production of Metal*

For this purpose the carbothermic reduction of columbium oxide to produce columbium metal has been chosen. The reaction in accordance with the equation is as follows:



The electrodes for this process are fabricated in accordance with the general techniques such as are described in our previous Letters Patent Number 2,616,842.

As a specific example, a formulation for the electrodes which were used for making columbium is:

3000 grams, —100 mesh calcined  $Cb_2O_5$   
356.7 grams, —325 mesh coke flour (e.g. 99% C coke of the Wilson Coke & Chemical Co.)  
149.1 grams liquid pitch paint (e.g. eternium paint of the Allied Chemical Corp.)

The columbium oxide and coke were dry mixed for one-half hour in a laboratory mix-muller. The liquid pitch paint was slowly added and the mixing continued for an additional one-half to three-quarters of an hour. The plastic mix was loaded into the cylinder of an extrusion press, de-aired, and extruded into convenient lengths at an extrusion pressure of 2750 p.s.i. The extruded electrodes were inserted into graphite tubes which were stacked in a stainless steel tray, covered with coke flour, and baked. During the baking operation, the loaded tray was inserted into an electric furnace and heated at a rate of 100° C. per hour to 900° C. and held about four hours at 900° C. to complete the baking process. The baked electrodes were straight, smooth and hard, with excellent compressive strength. Electrical resistivities in the order of .05 ohm-centimeters and densities in the order of 4.23 grams per cc. were achieved.

These electrodes were inserted into the feed mechanism of the arc chamber and the vessel was then pumped down to the order of 1000 microns pressure or less. The arc was then struck by contacting the anode with the cathode and retracting the cathode to its operating position.

Typical values of the operative conditions are given in the following:

|                                   |         |               |
|-----------------------------------|---------|---------------|
| Electrode diameter                | inches  | 3/4           |
| Carbon content of baked electrode | percent | 14.68 to 18.4 |
| Arc current                       | amperes | 40 to 60      |
| Arc voltage                       | volts   | 80 to 100     |
| Arc gap                           | inches  | 1 to 2        |
| Ambient pressure                  | microns | 300 to 1500   |
| Anode rotation rate               | r.p.m.  | 8 to 20       |

The best results in the laboratory were attained by using a 2" diameter homogeneous cathode of the same composition as the anode which was 3/4" diameter.

The process of making columbium metal from its oxide produced the metal in the form of spheres 1/4 to 5/16" diameter of 99.8% purity.

(B) *Production of Metal Carbide*

This is illustrated by the production of uranium monocarbide from uranium dioxide. The equation for this reaction is given specifically by:



The procedure for fabricating electrodes with uranium dioxide and carbon is essentially the same as that described above for columbium, except for the proportions

of ingredients. For example, we have used the formulation as follows:

1135 grams, —100 mesh uranium dioxide  
105.5 grams, —325 mesh coke flour  
149.1 grams, liquid pitch paint

For best results it was also found desirable to alter the baking schedule slightly whereby the green electrodes were fired by raising the furnace temperature initially at 10 a rate of 50° C. per hour until a temperature of 700° C. was reached. Subsequently the temperature was raised at a rate of 100° C. per hour until the maximum temperature of 900° C. was achieved; the temperature was then held at 900° C. for four hours.

The arc burning procedure followed that described for columbium metal except for the precise values of the operating parameters. Values used in the laboratory for producing UC are given in the following:

|                                   |         |             |
|-----------------------------------|---------|-------------|
| Electrode diameter                | inches  | 3/4         |
| Carbon content of baked electrode | percent | 11.8 to 12  |
| Arc current                       | amperes | 60 to 100   |
| Arc voltage                       | volts   | 40 to 60    |
| Ambient pressure                  | microns | 200 to 1500 |
| Anode rotation rate               | r.p.m.  | 8 to 20     |

The resulting product consisted of spheres of uranium monocarbide, having a purity as high as 99.9% and a density of 13.63 grams per cc.

What we claim is:

1. A process of reducing an oxide ore which comprises forming an anode of carbon and a stoichiometric quantity of ore to produce the metal product desired, maintaining a hierarc between a cathode and said anode, while limiting the temperature of the anode face at the arc crater to a point between the boiling point and the melting point of the metal product, whereby the said metal product accumulates in molten form upon the face of the anode until it drips off, while the other products are carried into the arc as vapors.

2. A process according to claim 1, in which the temperature of the crater is controlled by moving the anode face transverse to the arc terminus so that cooler anode material is continuously presented to the arc.

3. A process according to claim 1, in which the anode is in the form of a cylinder larger than the arc crater, which cylinder is rotated about its axis and the arc crater is on the end of the cylinder on one side of the axis.

4. A process according to claim 1, in which the anode is in the form of a cylinder larger than the arc crater, which cylinder is rotated about its axis and the arc crater is on the end of the cylinder on one side of the axis, by varying the current fed to the arc relative to the speed of rotation.

5. A process of conducting and controlling a hierarc to recover values from an ore which comprises establishing a hierarc between a cathode and an anode containing the ore and carbon, said anode having greater surface area than the hierarc crater to be established, striking 60 such an arc with said anode to form a crater while continuously moving said anode to cause the crater to change its position continuously, to maintain the temperature of the crater below the vaporizing temperature of the metal values.

6. The process of producing a metallic product in the form of spherical shot which comprises fabricating an anode comprising a mixture of carbon with metal-containing ore, establishing a hierarc with said anode to form a crater while continuously moving the position of said 70 crater so as to maintain the tip of the anode between the melting and boiling points of the product sought.

7. The process of reducing an ore which comprises forming an electrode of said ore with a quantity of carbon sufficient to reduce the ore to form the product desired, establishing a hierarc between a cathode and said

electrode as anode in an inert gas, whereby said ore is reduced at the anode face by the heat of the arc, while maintaining the temperature at the anode face above the melting point but below the vaporization temperature of the product.

## References Cited in the file of this patent

- Johnson et al.: "Arcs in Inert Atmospheres and Vacuum" (1956), pages 25 and 26.  
The High Intensity Electric Arc and Its Application to Process Chemistry, May 25, 1956, pages 20 and 22.